

## UNITED STATES PATENT OFFICE

2,274,025

## LUBRICANT

John S. Yule, Chicago, Ill., assignor to The Pure  
Oil Company, Chicago, Ill., a corporation of  
Ohio

No Drawing. Application December 28, 1940,  
Serial No. 372,185

22 Claims. (Cl. 252—48)

This invention relates to improvements in lubricants and more particularly to the method of improving mineral oil lubricants and to the product resulting therefrom.

Mineral lubricating oils, during use in internal combustion engines, tend to oxidize and corrode the bearings. The extent of corrosion varies with the type of bearing, the character of service and temperature to which the oil is subjected, and the particular oil used. Solvent refined Pennsylvania oils appear to be more corrosive than other oils which are not solvent refined, apparently due to the fact that the solvents remove natural inhibitors from the oil.

In addition to forming acids and corroding bearings, the oil has a tendency to form sludge and varnish which deposit on the various parts of the engine and not only cause faulty operation of the valves and other working parts, but in some cases cause sticking to such an extent that the motor entirely fails to operate. Such deposits are particularly apt to form when make-up oil is added to the engine. The make-up oil precipitates sludge and varnish from suspension or solution in the oil in the crankcase.

In order to prevent bearing corrosion and sludge and varnish formation in internal combustion engines, it has been proposed to add oxidation inhibitors to inhibit oxidation, and detergents to keep sludge and varnish dispersed in the oil and prevent it from depositing on the working parts of the motor. This invention is concerned with a novel inhibitor which has the ability to greatly inhibit oxidation of lubricating oil during use and reduce bearing corrosion.

It is known that phosphorized and sulfurized fatty oils and other fatty bodies have the ability of imparting extreme pressure characteristics to mineral oil lubricants when added thereto in amounts ranging upwardly from approximately 5%. I have now discovered that when compositions of this nature are added to mineral oil lubricants in relatively small amounts—that is, in amounts below that required to increase load-carrying ability of the oil to the extent necessary for use in connection with operation of gears, particularly hypoid gears—the compositions have the ability of inhibiting corrosion of bearings by otherwise corrosive mineral oils and of inhibiting oxidation, sludge and varnish formation of such mineral oils during use.

It is an object of this invention to provide a novel inhibitor for lubricating oils.

It is another object of this invention to provide a lubricating oil for use in internal com-

bustion engines which is inhibited against bearing corrosion and varnish formation.

It is still another object of this invention to provide a method of lubricating internal combustion engines with mineral lubricating oil in the presence of a novel oxidation inhibitor.

It is still a further object of this invention to minimize bearing corrosion and varnish formation in automotive engines.

10 Other objects of the invention will become apparent from the following detailed description.

In accordance with the invention, fatty bodies, including the higher boiling fatty acids and esters thereof, preferably fatty esters of low unsaturation such as rape seed, cotton, lard, sperm and other vegetable, animal or marine oils and waxes, are sulfurized and phosphorized. The method for accomplishing the sulfurization and phosphorization of the fatty body and the characteristics of the resulting products are described in the patent to William A. Whittier, Norman D. Williams and Harry L. Moir, No. 2,211,306. It will be understood, however, that there are other methods of preparing a sulfurized and phosphorized fatty body and that the composition contemplated by this invention includes sulfurized and phosphorized fatty bodies which may contain other elements such as chlorine and/or nitrogen. For example, in preparing the sulfurized and phosphorized fatty bodies, sulfur chloride may be used entirely as the sulfurizing agent instead of elemental sulfur and the reaction may be carried out under such conditions that both sulfur and chlorine remain combined with the fatty body and the resulting composition is then phosphorized. This can be done by adding from 3% to 15% by volume of sulfur chloride to the fatty body, maintaining the mixture between 145° and 155° F. until the exothermic reaction ceases, and then maintaining the mixture between 275° and 300° F. until it shows a good copper strip corrosion test. The resulting product is then phosphorized as set forth in Patent No. 2,211,306. This method of sulfurizing and phosphorizing fatty bodies is described in Whittier et al., application Serial Number 353,840.

When the sulfurized and phosphorized fatty material is added to mineral oil lubricants which normally have a tendency to corrode bearing surfaces and to oxidize and form acid, sludge and varnish in the motor, the corrosion, acid, sludge and varnish formation tendencies are remarkably inhibited. The effect of the sulfur-

ized-phosphorized base is particularly noticeable in connection with lubricating oils under high temperature or other severe operating conditions, particularly in connection with highly refined Pennsylvania base lubricating oils. Such oils are known to exert harmful corrosion under such conditions of operation on silver-cadmium, copper-lead and some other types of bearings. However, the invention is not limited to the use of the sulfurized-phosphorized base in connection with such oils since it has been found to have inhibiting properties in connection with practically all known types of lubricating oils.

In order to demonstrate the ability of the sulfurized-phosphorized fatty body to inhibit corrosion, sludge and varnish formation, various blends were subjected to Underwood corrosion tests. Experience has shown that the Underwood machine correlates actual service results rather closely. The Underwood test is described in an article entitled, "Automotive bearing materials and their application," by A. F. Underwood, Journal of Society of Automotive Engineers, volume 43, pages 385-392 (September, 1938).

A series of Underwood tests was run on straight 180 viscosity Pennsylvania neutral oil alone and to which was added different amounts of the sulfurized and phosphorized lard oil inhibitor, indicated as S-P lard oil, and sulfochlorinated and phosphorized lard oil, indicated as S-Cl-P lard oil, made as hereinbefore described. This series of tests was also run for five hours at 325° F. with 10#/sq. in. gauge oil pressure using .12% of iron naphthenate containing 0.01% by weight of iron calculated as  $Fe_2O_3$  as an oxidation catalyst to accelerate the tests. The results are given in Table I.

Table I

| Additive             | Loss in wt.<br>Ag. Cd. Brg. | Loss in wt.<br>Cu. Pb. Brg. | Neut.<br>No. | Naphtha,<br>insoluble |
|----------------------|-----------------------------|-----------------------------|--------------|-----------------------|
| 180 vis. Pa. neut.   | 0.796                       | 0.080                       | 11.9         | 1.62                  |
| 0.5% S-P lard oil    | 0.036                       | 0.038                       | 1.5          | 0.67                  |
| 1.0% S-P lard oil    | 0.012                       | 0.015                       | 2.1          | 0.52                  |
| 1.5% S-P lard oil    | 0.003                       | 0.015                       | 1.1          | 0.46                  |
| 2.0% S-P lard oil    | 0.0003                      | 0.002                       | 1.3          | 0.32                  |
| 2.5% S-P lard oil    | 0.005                       | 0.014                       | 0.91         | 0.62                  |
| 3.0% S-P lard oil    | 0.003                       | 0.011                       | 0.4          | 0.31                  |
| 5.0% S-P lard oil    | 0.001                       | 0.031                       | 0.61         | 0.16                  |
| 7.0% S-P lard oil    | 0.002                       | 0.080                       | 0.48         | 0.17                  |
| 1.0% S-Cl-P lard oil | 0.0058                      | 0.0620                      | 0.60         | 0.45                  |
| 3.0% S-Cl-P lard oil | 0.0009                      | 0.0048                      | 0.51         | 0.12                  |
| 5.0% S-Cl-P lard oil | 0.0033                      | 0.0238                      | 0.70         | 0.52                  |

| Additive                | Chloroform<br>soluble | Soluble<br>sludge |
|-------------------------|-----------------------|-------------------|
| 180 vis. Pa. neut.      | Per cent              | Per cent          |
| 0.5% S-P lard oil       | 1.24                  | 5.29              |
| 1.0% S-P lard oil       | 0.36                  | 1.09              |
| 1.5% S-P lard oil       | 0.29                  | 1.89              |
| 2.0% S-P lard oil       | 0.13                  | 1.32              |
| 2.5% S-P lard oil       | 0.13                  | 1.28              |
| 3.0% S-P lard oil       | 0.23                  | 1.10              |
| 5.0% S-P lard oil       | 0.09                  | 0.57              |
| 7.0% S-P lard oil       | 0.04                  | 1.28              |
| 1.0% of S-Cl-P lard oil | 0.04                  | 2.06              |
| 3.0% of S-Cl-P lard oil | 0.33                  | 0.51              |
| 5.0% of S-Cl-P lard oil | 0.03                  | 0.62              |
|                         | 0.23                  | 1.10              |

The 180 vis. Pennsylvania neutral was examined prior to being run on the Underwood machine and gave the results indicated in Table II:

Table II

| Nature of oil                            | Neut.<br>No. | Naphtha<br>insoluble | Chloroform<br>soluble | Soluble<br>sludge |
|------------------------------------------|--------------|----------------------|-----------------------|-------------------|
| 180 vis. neut.                           | 6.0          | Per cent<br>0.97     | Per cent<br>0.04      | Per cent<br>0.17  |
| 180 vis. neut.+0.12%<br>iron naphthenate | 0.09         | 0.125                | 0.07                  | 0.20              |

10 The "naphtha insoluble" is an indication of the amount of insoluble sludge formed by the oil during the test. The "chloroform soluble" portion indicates the varnish formation which took place during the test; and the neutralization or acid number is a measure of the total acidity of the oil.

15 The acid or neutralization number is determined in accordance with A. S. T. M. tentative method D188-27T.

20 The "naphtha insoluble," "chloroform soluble" and "soluble sludge" are determined as follows:

#### Naphtha insoluble (insoluble sludge)

25 Three grams of the oil is mixed in an Erlenmeyer flask with 100 cc. of A. S. T. M. precipitation naphtha, of the type specified in A. S. T. M. method D91-35. The oil and naphtha are thoroughly mixed and allowed to stand for 3 hours. The insoluble matter is then filtered through a tared Gooch porcelain crucible, previously prepared with an asbestos pad 1" thick and dried in an oven at 300° F. for 30 minutes. The insoluble residue is washed with 100 cc. A. S. T. M. naphtha and dried in an oven at 300° F. for 30 minutes, cooled and weighed. The increase in weight is "naphtha insoluble."

#### Chloroform soluble

40 The chloroform soluble is extracted from the dried and weighed "naphtha insoluble" residue by pouring successive portions of chloroform through the filter pad using light suction. 100 cc. of chloroform is generally sufficient but the extraction should be continued until the filtrate is colorless. (With heavy "naphtha insoluble" residues the chloroform is allowed to stand in the crucible without suction for a few minutes before each portion of the chloroform is drawn through the crucible.)

45 The residue is then dried in an oven at 300° F. for 30 minutes, cooled and weighed. The loss in weight is "chloroform soluble."

50 The solubility in chloroform of the residue from the "naphtha insoluble" determination is affected by the time and temperature of drying. For this reason, in order to secure check results in the "chloroform soluble" determination, the drying time and temperature, especially in the "naphtha insoluble" determination, should be carefully controlled.

60 It usually happens that in the Underwood test there is no particular difficulty in filtering, regardless of whether the oils contain detergents or not. However, when these methods are applied to used crankcase oils it sometimes happens that oils which contain detergents will not give a clear filtrate. Under these conditions, the filtrate is re-filtered through a second Gooch filter and the deposits from both crucibles added in reporting naphtha insoluble (and chloroform soluble).

#### Propane soluble (soluble sludge)

65 The filtrate from the naphtha insoluble is concentrated to 20 cc. by evaporation and is trans-

ferred quantitatively to the extraction apparatus described in Industrial & Engineering Chemistry, April 15, 1939, page 183. The remaining naphtha is now completely removed from the oil sample by evaporation on a steam bath. The propane extraction is carried out as directed in the above-mentioned article. The propane insoluble material remaining is calculated in percentage and reported as soluble sludge.

It will be seen that the corrosion of both the silver-cadmium and copper-lead bearings was materially decreased by addition of the sulfurized-phosphorized fatty body and that the acid-forming, sludge and varnish-forming tendencies were likewise remarkably decreased. The effectiveness of the S-P lard oil base was particularly noticeable when added in the proportion of from 2% to 3% by volume. The oil containing 2% of the base was the least corrosive, whereas the oil containing 3% of the base formed the least amount of acid, varnish and sludge. The optimum amount of additive is, therefore, between 2-3% by volume. Approximately 3% also appears to be the optimum for the S-Cl-P lard oil inhibitor. No advantage is gained by exceeding 5% by weight of the inhibitor since both corrosion and sludge formation are less below than above 5%.

A series of tests were also made on blends of straight 180 viscosity Pennsylvania neutral with sulfurized-phosphorized lard oil and a commercial lubricating oil detergent prepared by reacting tin diphenyl oxide with lauric acid. The results on these tests showing the loss in weight in silver-cadmium bearings and copper-lead bearings on the Underwood machine and the examination of the oil after the tests are set forth in Table III:

Table III

|                                          | 180 vis. oil (straight) | 180 vis. oil + 1% S-P lard oil and .5% detergent | 180 vis. oil + 1.5% S-P lard oil and .5% detergent | 180 vis. oil + 3% S-P lard oil and .5% detergent | Straight 180 vis. Pa. + .5% detergent |
|------------------------------------------|-------------------------|--------------------------------------------------|----------------------------------------------------|--------------------------------------------------|---------------------------------------|
| Loss in weight of silver-cadmium bearing | 0.796                   | 0.282                                            | 0.344                                              | 0.351                                            | 0.366                                 |
| Loss in weight of copper-lead bearing    | 0.080                   | 0.158                                            | 0.047                                              | 0.080                                            | 0.224                                 |
| Neutralization No.                       | 11.9                    | 1.13                                             | 3.36                                               | 1.80                                             | 1.82                                  |
| Naphtha insoluble, percent               | 1.62                    | 0.22                                             | 1.26                                               | 0.97                                             | 0.55                                  |
| Chloroform insoluble                     | do                      | 1.24                                             | 0.13                                               | 0.62                                             | 0.38                                  |
| Soluble sludge                           | do                      | 5.29                                             | 0.69                                               | 3.53                                             | 1.74                                  |

The same 180 vis. Pennsylvania neutral was subjected to the Chevrolet engine test without any inhibitor but containing 0.5% of the same detergent used in the Underwood tests and also with the detergent plus 1.5% of the S-P lard oil inhibitor previously described. The results are set forth in Table IV:

Table IV

| Oil                                                     | Neut. No. | Bearing cap half | Loss in grs. rod half |
|---------------------------------------------------------|-----------|------------------|-----------------------|
| 180 vis. Pa. neut. + 0.5% detergent                     | 1.84      | .26              | .27                   |
| 180 vis. Pa. neut. + 0.5% detergent + 1.5% S-P lard oil | 1.18      | .06              | 1.02                  |

<sup>1</sup> Gain.

The Chevrolet engine test is run as follows: The engine is operated at a speed of 3150 R. P. M., equivalent to 60 miles per hour. A dynamometer load is applied equivalent to 25 to 30 horsepower. The oil sump temperature is maintained at 280° F. plus or minus 2° F. and the cooling water out is maintained at 200° F. plus or minus 2° F. The test is run for 66½ hours

with no oil change during the entire test. The test is started with 5 quarts of oil.

In starting the test, the engine is run for about 10 minutes at 2000 R. P. M. and 15 to 25 horsepower until the oil reaches 150° F. The speed is then increased to 3150 R. P. M. and run until the oil temperature reaches 280° F., at which time the test is considered to have begun. Oil is added one quart at a time as needed, but no oil is added during the last 400 miles, or 6½ hours of the run.

From Tables III and IV it will be observed that by proper balancing of the amount of detergent and inhibitor added to the oil, bearing corrosion can be considerably reduced below that amount which occurs when straight oil or oil plus detergent only are used. The tables also show that although the bearing loss of the oil containing inhibitor and detergent was less than in the case of the straight oil without both inhibitor and detergent, the loss in weight of the bearings as well as the neutralization number, naphtha insoluble, chloroform soluble and soluble sludge were all higher in the case where both the detergent and the sulfurized-phosphorized base were used than in the case where only the sulfurized-phosphorized lard oil inhibitor was used. An examination of the engine parts at the conclusion of the test showed, however, that the deposits were noticeably less in the case where the detergent was used than in the case where no detergent was used. Thus, although the detergent appears to somewhat detract from the inhibitory powers of the S-P base, it is, nevertheless, beneficial to the engine to use detergent in conjunction with the base in order to prevent deposition of varnish on the working parts of

the engine. This is particularly true in connection with Diesel engine operations where because of the high pressures used, the blow-by past the piston rings is comparatively large and as a result more oxidation and varnish formation in the oil take place. With present compression ratios in spark ignition type automotive engines, the use of the detergent in conjunction with the sulfurized-phosphorized fatty base inhibitor is not so essential since oxidation, because of the small amount of blow-by, is almost entirely avoided by the sulfurized-phosphorized lard oil base and therefore, varnish formation is not particularly troublesome.

Thus, although the sulfurized-phosphorized fatty base cuts down sludge and varnish formation, there will be some amount of sludge and varnish formation, the amount depending upon the conditions of operation of the engine, the particular engine in connection with which the oil is used and the particular oil used. Deposition of this varnish on the working parts should be prevented by addition of a proper detergent in order to have the engine operate efficiently. It will be understood that detergents other than

the specific detergent above named may be used and such detergents may be added in amounts approximately those of the inhibitor.

A series of Timken and Faville-Levalley (Falex) tests were also run in order to indicate whether or not the sulfurized-phosphorized base had any substantial extreme pressure load imparting characteristics when added to mineral oil in small proportions. The results of these tests are given in the following table:

Table V

| Oil                        | S-P lard oil in blend | Timken    |             | Falex  |
|----------------------------|-----------------------|-----------|-------------|--------|
|                            |                       | Beam load | Max. press. |        |
| Gulf Coast oil S. A. E. 90 | Percent               | Pounds    | #/sq. in.   | Pounds |
| Do.                        | 0.5                   | 8         | 4,500       | 750    |
| Do.                        | 1.0                   | 12        | 6,150       | 1,250  |
| Do.                        | 2.0                   | 18        | 7,750       | 1,450  |
| Do.                        | 2.5                   | 18        | 8,250       | 1,600  |
| Do.                        | 3.0                   | 18        | 10,250      | 1,750  |
| Do.                        | 5.0                   | 43        | 20,000      | 1,850  |
| Do.                        | 7.0                   | 43        | 24,500      | 2,000  |
| Do.                        | 10.0                  | 43        | 27,750      | 2,250  |
| Do.                        | 18.0                  | 68        | 35,000      | 3,000  |
| 180 vis. Pa. neutral       |                       | 5         | 4,200       | 500    |
| Do.                        | 0.5                   | 8         | 4,570       | 1,525  |
| Do.                        | 1.0                   | 12        | 7,250       | 1,500  |
| Do.                        | 2.0                   | 18        | 8,250       | 1,600  |
| Do.                        | 2.5                   | 18        | 8,750       | 1,600  |
| Do.                        | 3.0                   | 18        | 8,750       | 1,600  |
| Do.                        | 5.0                   | 18        | 10,250      | 1,750  |
| Do.                        | 7.0                   | 25        | 18,500      | 1,750  |
| Do.                        | 10.0                  | 51        | 23,000      | 2,100  |
| Do.                        | 18.0                  | 68        | 33,250      | 2,200  |

An oil is not considered to be a satisfactory commercial extreme pressure lubricant unless it will hold a pressure of at least 25,000#/sq. in. on the Timken machine and at least 2500 lbs. on the Falex machine. It will be apparent, therefore, that the inhibitor is effective as such in amounts in which it has little value as an extreme pressure additive.

Timken and Falex tests were also made on a sulfochlorinated and phosphorized lard oil prepared in the manner previously described. The results are set forth in Table VI:

Table VI

| Oil                        | 12% S-Cl-P lard oil in blend | Timken at 800 r. p. m. |             | Falex max. load                                              |
|----------------------------|------------------------------|------------------------|-------------|--------------------------------------------------------------|
|                            |                              | Beam load              | Max. press. |                                                              |
| Gulf coast oil S. A. E. 90 |                              | Pounds                 | #/sq. in.   |                                                              |
| Do.                        | 1                            | 25                     | 14,250      | 750# (journal sheared).                                      |
| Do.                        | 3                            | 33                     | 21,250      | 1,500# (brass pin sheared).                                  |
| Do.                        | 5                            | 43                     | 15,000      | 1,500# (brass pin sheared).                                  |
| Do.                        | 7                            | 43                     | 15,500      | 1,650# (brass pin sheared).<br>1,750# (would not hold load). |
| Do.                        | 10                           | 43                     | 20,000      | 1,750# (would not hold load).                                |
| Do.                        | 12                           | 43                     | 24,500      | 4,500# (full load).                                          |
| Do.                        | 16                           | 51                     | 29,250      | 4,500# (full load).                                          |
| Do.                        | 18                           | 51                     | 29,250      | 4,500# (full load).                                          |
| 180 vis. Pa. neutral       |                              | 5                      | 4,200       | 500# (journal sheared).                                      |
| Do.                        | 1                            | 18                     | 9,250       | 1,600# (brass pin sheared).                                  |
| Do.                        | 3                            | 33                     | 13,000      | 1,600# (brass pin sheared).                                  |
| Do.                        | 5                            | 43                     | 17,000      | 1,888 (brass pin sheared).                                   |
| Do.                        | 7                            | 43                     | 20,000      | 1,900 (brass pin sheared).                                   |
| Do.                        | 10                           | 51                     | 26,000      | 4,500 (brass pin sheared).                                   |
| Do.                        | 12                           | 51                     | 26,000      | 4,500 (brass pin sheared).                                   |
| Do.                        | 16                           | 51                     | 29,250      | 4,500 (brass pin sheared).                                   |
| Do.                        | 18                           | 51                     | 31,000      | 4,500 (brass pin sheared).                                   |

In view of the fact that an oil is not considered to be a satisfactory commercial extreme pressure lubricant unless it will carry a load on the Timken machine above 25,000#/sq. in. and above 2500# on the Falex machine, it will be seen that the sulfo-chlorinated phosphorized fatty mate-

rial is an effective inhibitor when used in amounts below that at which it is an effective extreme pressure additive.

It will be seen, therefore, that the sulfurized-phosphorized fatty material has unusual properties in imparting to mineral oils corrosion resistant properties and resistance to acid, sludge and varnish formation. The inhibitor may be added to the mineral oil alone or to oils to which have been added other materials such as detergents. Although I have found that the optimum amount of inhibitor which should be added to the mineral oil is between approximately 2-3% by volume, beneficial results may be obtained with amounts as low as 0.1% by volume. The tests indicate that there is no advantage in adding in excess of 5% by volume of the inhibitor where the oil is to be used for lubrication of internal combustion engines. Thus, it will be seen that the sulfurized-phosphorized fatty material when added to mineral oil lubricants in quantities so small as to not be practicable as an extreme pressure additive, is valuable in inhibiting corrosion of bearings and in stabilizing the oil during use in a motor and in connection with lubrication of other bearing surfaces.

It is claimed:

1. A lubricant comprising mineral lubricating oil and between 0.1 and 5% by volume of sulfurized and phosphorized fatty material.
2. A lubricant in accordance with claim 1 in which the fatty material is lard oil.
3. A lubricant in accordance with claim 1 in which the fatty material is sperm oil.
4. A lubricant in accordance with claim 1 in which the fatty material is rapeseed oil.
5. A lubricant in accordance with claim 1 in which the sulfurized and phosphorized fatty material contains from 2% to 7% by weight of sulfur and from 0.11% to 0.56% by weight of phosphorus.
6. The method of inhibiting corrosion of metallic bearings and deterioration of lubricating oils in service which comprises contacting said bearing with mineral oils which normally tend to

corrode said bearing and to deteriorate during use, in the presence of from 0.1% to 5% by volume of sulfurized and phosphorized fatty material.

7. Method in accordance with claim 6 in which the fatty material is lard oil.

8. Method in accordance with claim 6 in which the fatty material is sperm oil.
9. Method in accordance with claim 6 in which the fatty material is rapeseed oil.
10. Method in accordance with claim 6 in which the sulfurized and phosphorized fatty material contains from 2% to 7% of sulfur and from 0.11% to 0.56% by weight of phosphorus.
11. The method of lubricating internal combustion engines which comprises contacting the moving parts thereof with a mineral lubricating oil containing sufficient sulfurized and phosphorized fatty material to inhibit oxidation of said oil but insufficient to materially increase the viscosity of said oil.
12. Method in accordance with claim 11 in which the sulfurized and phosphorized fatty material is present in amounts of 0.1% to 5% by volume.
13. Method in accordance with claim 11 in which the fatty material is lard oil.
14. Method in accordance with claim 11 in which the fatty material is sperm oil.
15. Method in accordance with claim 11 in which the sulfurized and phosphorized fatty material is prepared by reacting a fatty body with sulfur chloride and with a reactive phosphorus compound.
16. Method in accordance with claim 11 in which the sulfurized and phosphorized fatty material contains from 2% to 7% by weight of sulfur and from 0.11% to 0.56% by weight of phosphorus.
17. Method in accordance with claim 11 in which the sulfurized and phosphorized fatty material is prepared by reacting lard oil with sulfur at elevated temperature and then reacting the sulfurized lard oil with a phosphorus containing material capable of chemically uniting phosphorus with the sulfurized lard oil.
18. A lubricant comprising mineral lubricating oil, between 0.1% and 5% by volume of sulfurized and phosphorized fatty material and a small amount of a detergent.
19. The method of lubricating internal combustion engines which comprises contacting the working parts of said engines with mineral lubricating oil in the presence of a small amount of sulfurized and phosphorized fatty material and a small amount of a detergent.
20. Method in accordance with claim 19 in which the sulfurized and phosphorized fatty material is present in amounts of from 0.1% to 5% by volume of the oil.
21. A lubricant in accordance with claim 1 in which the fatty material is sulfurized by reacting between approximately 3% and 15% of sulfur halide therewith.
22. Method in accordance with claim 6 in which the fatty material is sulfurized by reacting between approximately 3% to 15% of sulfur halide therewith.

JOHN S. YULE.